

# UNITED STATES PATENT OFFICE.

MICHAEL M. KLINE, OF ST. LOUIS, MISSOURI.

## ARTIFICIAL-FUEL BLOCK AND METHOD OF PRODUCING SAME.

No. 850,232.

Specification of Letters Patent.

Patented April 16, 1907.

Application filed July 30, 1906. Serial No. 328,362.

To all whom it may concern:

Be it known that I, MICHAEL M. KLINE, a citizen of the United States, residing at St. Louis, Missouri, have invented a certain new and useful Improvement in Artificial-Fuel Blocks and Methods of Producing Same, of which the following is a full, clear, and exact description, such as will enable others skilled in the art to which it appertains to make and use the same.

This invention relates to artificial-fuel blocks.

One object of my invention is to provide a fuel-block which is harder and contains a greater percentage of fuel and is superior in a number of other ways to the artificial-fuel blocks heretofore in use.

Another object of my invention is to provide a novel method of producing artificial fuel blocks.

The fuel-block herein described as embodying my invention may be of any desired form or size, and consists of the following ingredients of about the proportions specified: 25 pulverized slack coal, ninety-seven and three-fifths per cent.; starch, one per cent.; glucose, one per cent.; sulfate of iron, one-fifth of one per cent.; sulfate of magnesia, one-tenth of one per cent.; oxid of manganese, one-tenth of one per cent.

While I have herein stated that my fuel-block consists of ingredients of about the proportions specified, I wish it to be understood that these are about the maximum proportions, as the condition of the coal-slack which is used determines the proportions of the other ingredients. I prefer to use starch and glucose to act as the binding agent; but oatmeal or any other farinaceous 35 substance could be used equally well.

The method of producing the article consists in thoroughly mixing pulverized slack coal, glucose, starch, sulfate of iron, sulfate of magnesia, and oxid of manganese of about 45 the proportions previously specified with enough water to make the mass plastic and cause the ingredients to mix thoroughly, then heating the mass and molding a proper quantity thereof into the desired form by 50 subjecting it to great pressure between heated dies. The sulfate of iron, sulfate of magnesia, and oxid of manganese harden the block and also destroy the smoke, and thus aid combustion. The block is clean and is so

very hard that it can be handled readily and transported without liability of breakage. In some ways it is superior to hard coal, as it is completely consumed in burning, it gives off no smoke, and leaves no clinker.

The cost of producing the block is only a fraction of the cost of a good grade of hard coal, as either bituminous or anthracite slack or culm or lignite coal can be used.

Having thus described my invention, what I claim as new, and desire to secure by Letters Patent, is—

1. An artificial-fuel block comprising pulverized slack coal, a binding agent, sulfate of iron, sulfate of magnesia and oxid of manganese intimately mixed with each other and compressed into a solid mass; substantially as described.

2. An artificial-fuel block comprising ninety-seven and three-fifths per cent. of pulverized slack coal, one per cent. of starch, one per cent. of glucose and one-fifth of one per cent. of sulfate of iron, one-tenth of one per cent. of sulfate of magnesia and one-tenth of one per cent. of oxid of manganese intimately mixed with each other and compressed into a solid mass; substantially as described.

3. The method of producing an artificial-fuel block which consists in mixing pulverized slack coal, a binding agent, and a hardening and smoke-destroying substance with a liquid to form a plastic mass, heating said mass and then subjecting a portion thereof to great pressure and to heat to mold it into predetermined form; substantially as described.

4. The method of producing an artificial-fuel block which consists in mixing pulverized slack coal, glucose, starch, sulfate of iron, sulfate of magnesia, oxid of manganese with enough water to cause the ingredients to mix thoroughly, heating the mass and then subjecting a portion thereof to great pressure between heated members to mold it into predetermined form; substantially as described.

In testimony whereof I hereunto affix my signature, in the presence of two witnesses, this 20th day of July, 1906.

MICHAEL M. KLINE.

Witnesses:

WELLS L. CHURCH,  
CORA BADGER.